



US005998118A

# United States Patent [19]

Schwark et al.

[11] Patent Number: **5,998,118**[45] Date of Patent: **Dec. 7, 1999**

[54] **BACKSIDE PROTECTIVE OVERCOAT COMPOSITIONS FOR SILVER HALIDE PHOTOGRAPHIC ELEMENTS**

[75] Inventors: **Dwight W. Schwark**, Rochester; **Yongcui Wang**; **Charles C. Anderson**, both of Penfield, all of N.Y.

[73] Assignee: **Eastman Kodak Company**, Rochester, N.Y.

[21] Appl. No.: **09/019,065**

[22] Filed: **Feb. 5, 1998**

[51] **Int. Cl.<sup>6</sup>** ..... **G03C 1/89**; G03C 1/93; G03C 1/76

[52] **U.S. Cl.** ..... **430/529**; 430/527; 430/536; 430/961

[58] **Field of Search** ..... 430/536, 961, 430/527, 529

## [56] References Cited

### U.S. PATENT DOCUMENTS

4,582,784 4/1986 Fukugawa et al. ..... 430/536  
4,612,279 9/1986 Steklenski et al. ..... 430/536

4,735,976 4/1988 Steklenski et al. ..... 524/32  
5,173,739 12/1992 Kurachi et al. ..... 356/124  
5,466,536 11/1995 Berner et al. ..... 430/536  
5,597,680 1/1997 Wang et al. ..... 430/536  
5,597,681 1/1997 Anderson et al. ..... 430/536  
5,695,919 12/1997 Wang et al. ..... 430/536  
5,786,135 7/1998 Anderson et al. ..... 430/536

### FOREIGN PATENT DOCUMENTS

476 535 8/1997 European Pat. Off. .

*Primary Examiner*—Richard L. Schilling  
*Attorney, Agent, or Firm*—Carl F. Ruoff

## [57] ABSTRACT

The present invention is a photographic element which includes a support having a frontside and a backside, at least one silver halide emulsion layer superposed on the frontside of the support; and a protective overcoat layer superposed on the backside of the support. The protective overcoat layer is a mixture of a first vinyl polymer having an acid number of from 5 to 100 and a second vinyl polymer having an acid number of from 70 to 250 wherein the acid number of the second polymer is greater than the acid number of the first polymer.

**13 Claims, No Drawings**

# BACKSIDE PROTECTIVE OVERCOAT COMPOSITIONS FOR SILVER HALIDE PHOTOGRAPHIC ELEMENTS

## FIELD OF THE INVENTION

The present invention relates to a photographic element with improved physical properties of its backside protective overcoat. In particular, the present invention relates to photographic elements having a backside protective overcoat which provides the elements with excellent barrier properties, excellent resistance to surface haze or scum formation and blistering during photographic processing, and excellent protection against mechanical scratch and high humidity ferrotyping.

## BACKGROUND OF THE INVENTION

Photographic light-sensitive materials are generally composed of light-sensitive photographic emulsion layers and light insensitive layers such as an interlayer, an emulsion protective layer, a filter layer, or an antihalation layer applied, directly or indirectly through a subbing layer, to one side or both sides of the support consisting of, for example, an  $\alpha$ -olefin such as polyethylene, a cellulose ester such as cellulose acetate or nitrocellulose, a polyester such as polyethylene terephthalate or polyethylene naphthalate, polystyrene, paper, or a synthetic paper. In light-sensitive materials such as color photographic elements, auxiliary layers such as an antistatic layer, a curl preventing layer, a magnetic recording layer, a barrier layer, a scratch resistant overcoat layer, or a surface lubricant layer, are provided on the backside of the support in order to enhance the photographic or physical quality of the photographic light-sensitive materials.

It is always desirable to have a backside protective overcoat that serves as many functions as possible in order to reduce manufacturing complexity and cost. It is also desirable to have such a layer formed by coating and drying from coating compositions based on solvents that are less hazardous to the environment.

Prior art has disclosed the use of a protective overcoat or a "barrier" layer to maintain post-process conductivity of an antistatic layer. Typically such protective overcoats consist of hydrophobic materials such as cellulose acetates, cellulose acetate butyrates, cellulose acetate propionates, cellulose nitrates, polyacrylates, polymethacrylates, polystyrene, and poly(vinyl acetal).

When such hydrophobic barrier layers are used as an outermost surface layer, deposition of material or "scum" formation on the outermost surface following photographic processing is commonly seen. For example, U.S. Pat. No. 4,735,976, incorporated by reference herein, discusses how surfactant from the final photographic processing solution, known as the stabilizer solution, can form a deposit on the outermost surface layer and thereby lead to an objectionable surface haze or scum. Similarly, U.S. Pat. No. 4,582,784, incorporated by reference herein, discusses the occurrence of spotted drying unevenness on the outermost surface. Another type of processing scum that is particularly troublesome is hard-water scum. Processing laboratories that are located in hard-water areas are particularly susceptible to this problem. After processing in solutions prepared using hard-water, a white hazy surface scum, sometimes uniform and sometimes more liney and streaky, can be seen on the film. Chemical analysis of the hard-water scum typically reveals hard-water salts of calcium, magnesium, and sodium.

Such surface deposits can impact the physical performance of the element in a variety of ways. For example, large deposits of material on a photographic film lead to readily visible defects on photographic prints or are visible upon display of motion picture film. Alternatively, post-processing debris can influence the ability of a processed film to be overcoated with an ultraviolet curable abrasion resistant layer, as is done in professional photographic processing laboratories employing materials such as PhotoGard, 3M. Finally, processing residue on photographic elements can impact the ability to read or write magnetically recorded information on a processed film, such as the new Advanced Photographic System film.

U.S. Pat. Nos. 4,612,279 and 4,735,976, incorporated by reference herein, describe a protective overcoat comprising a blend of cellulose nitrate and a copolymer containing acrylic or methacrylic acid for eliminating objectionable surface haze or scum formed during photographic processing. U.S. Pat. No. 4,582,784 describes an uppermost surface layer composed of a hydrophobic cellulose ester polymer and a hydrophilic vinyl polymer for reducing spotted drying unevenness. However, layer compositions disclosed in the above art do not provide adequate barrier properties and adequate resistance to mechanical scratch and high humidity ferrotyping. High humidity ferrotyping becomes a problem especially for photographic systems such as the so-called Advanced Photographic System where the processed element may be re-introduced into a cassette. Such a system allows for compact and clean storage of the processed element until such time when it may be removed for additional prints or to interface with display equipment. Storage in the roll is preferred to facilitate location of the desired exposed frame and to minimize contact with the negative. U.S. Pat. No. 5,173,739, incorporated by reference herein, discloses a cassette designed to thrust the photographic element from the cassette, eliminating the need to contact the film by mechanical or manual means. Published European Patent Application 0 476 535 A1 describes how the developed film may be stored in such a cassette. The dimensions of such a so-called thrust cassette require that the processed photographic element be wound tightly and under pressure, causing direct close contact between the front and back sides which results in ferrotyping, especially at high temperature and high relative humidity.

U.S. Pat. Nos. 5,597,680 and 5,597,681, incorporated by reference herein, describe a protective layer coating composition applied from a dispersion of core/shell polymer particles in a liquid organic medium. Such protective layers provide photographic elements with excellent barrier properties and excellent resistance to mechanical scratch and ferrotyping at high temperature and in moist environments. However, such coating compositions do not provide the photographic elements with adequate protection against surface haze or scum formation under more severe processing conditions.

Blisters are characteristic defects that are often observed on the backside of a developed film. When viewed by reflected light, the defect appears as a circular-shaped topographic feature with a wrinkled surface texture. The diameter of the blister can be as large as several millimeters. Blisters not only affect the photographic image quality, but also the read and write ability of a magnetic layer and the image digitization, for example, by a scanner.

The objective of the present invention is to provide a photographic element with a backside protective overcoat composition that meets all of the physical and mechanical requirements as described above while avoiding the problems and limitations of the prior art.

## SUMMARY OF THE INVENTION

The present invention is a photographic element which includes a support having a frontside and a backside, at least one silver halide emulsion layer superposed on the frontside of the support; and a protective overcoat layer applied from an organic solvent superposed on the backside of the support. The protective overcoat layer is a mixture of a first vinyl polymer having an acid number of from 5 to 100 and a second vinyl polymer having an acid number of from 70 to 250 wherein the acid number of the second polymer is greater than the acid number of the first polymer.

The photographic elements prepared in accordance with this invention have excellent antistatic properties, excellent resistance to scratch and ferotyping, and excellent resistance to surface haze or scum formation and blistering during photographic processing.

## DESCRIPTION OF THE INVENTION

The photographic elements of this invention can vary greatly in regard to the type of the support. Typical supports include cellulose nitrate film, cellulose acetate film, poly(vinyl acetal) film, polystyrene including syndiotactic polystyrene film, polycarbonate film, poly(ethylene terephthalate) film, poly(ethylene naphthalate) film, glass, metal plate, paper, polymer coated paper, and the like. The support may be annealed. The thickness of the support is not critical. Support thickness of 2 to 10 mils (0.002 to 0.010 inches) can be used. The supports typically employ an undercoat or subbing layer well known in the art that comprises, for example, for polyester support a vinylidene chloride/methyl acrylate/itaconic acid terpolymer or vinylidene chloridelacrylonitrile/acrylic acid terpolymer.

The present invention contemplates a photographic element that comprises a support, at least one silver halide emulsion layer superposed on the frontside of the support, and a protective overcoat layer on the backside of the support comprising a mixture of a first vinyl polymer having an acid number of from 5 to 100 and a second vinyl polymer having an acid number of from 70 to 250 wherein the acid number of the second polymer is greater than the acid number of the first polymer. The backside protective overcoat is applied from organic solvents. The acid number is defined as the number of milligrams of potassium hydroxide needed to neutralize one gram of polymer. Preferably the first vinyl polymer has an acid number of from 5 to 65, and the second vinyl polymer has an acid number of from 80 to 150. Also preferably the weight ratio of the second polymer to the first polymer ranges from 5:95 to 40:60, and more preferably from 5:95 to 30:70. There is no limitation on the molecular weight of the polymers. However, preferably the molecular weight of the second vinyl polymer is lower than that of the first vinyl polymer. Other additional compounds may be added to the coating composition, depending on the functions of the particular layer, including surfactants, coating aids, matte particles, rheology modifiers, crosslinking agents, inorganic fillers such as metal oxide particles, pigments, antistatic agents, magnetic particles, biocide, lubricants, and the like.

The amount of the total polymers applied in the backside protective overcoat is preferably in the range of from 0.01 to 10 g/m<sup>2</sup>, and more preferably from 0.1 to 2 g/m<sup>2</sup>.

The vinyl polymers useful for the present invention include those obtained by interpolymerizing one or more ethylenically unsaturated monomers containing carboxylic acid groups with other ethylenically unsaturated monomers including, for example, alkyl esters of acrylic or methacrylic

acid such as methyl methacrylate, ethyl methacrylate, butyl methacrylate, ethyl acrylate, butyl acrylate, hexyl acrylate, n-octyl acrylate, lauryl methacrylate, 2-ethylhexyl methacrylate, nonyl acrylate, benzyl methacrylate, the hydroxyalkyl esters of the same acids such as 2-hydroxyethyl acrylate, 2-hydroxyethyl methacrylate, and 2-hydroxypropyl methacrylate, the nitrile and amides of the same acids such as acrylonitrile, methacrylonitrile, and methacrylamide, vinyl acetate, vinyl propionate, vinylidene chloride, vinyl chloride, and vinyl aromatic compounds such as styrene, t-butyl styrene and vinyl toluene, dialkyl maleates, dialkyl itaconates, dialkyl methylenemalonates, isoprene, and butadiene. Suitable ethylenically unsaturated monomers containing carboxylic acid groups include acrylic monomers such as acrylic acid, methacrylic acid, ethacrylic acid, itaconic acid, maleic acid, fumaric acid, monoalkyl itaconate including monomethyl itaconate, monoethyl itaconate, and monobutyl itaconate, monoalkyl maleate including monomethyl maleate, monoethyl maleate, and monobutyl maleate, citraconic acid, and styrene carboxylic acid.

When the polymerization is carried out using a hydroxyl-containing monomer such as a C2-C8 hydroxyalkyl esters of acrylic or methacrylic acid, a vinyl polymer containing a hydroxyl group as well as a carboxyl group can be obtained.

It is preferred to incorporate in the vinyl polymers a certain amount of fluorinated or perfluorinated vinyl monomers. Such perfluorinated, ethylenically unsaturated monomers can contain a fluorocarbon group either directly bonded to an ethylenically unsaturated group or bonded to a hydrocarbon portion which is in turn bonded to an ethylenically unsaturated group. The bonding between the fluorocarbon group and the hydrocarbon portion may either be direct or through a bridging group such as a sulfonamido group. Examples of ethylenically unsaturated monomers are acrylate and methacrylate monomers. Typical fluorinated, ethylenically unsaturated monomers include:



60  $\text{C}_7\text{F}_{15}\text{COOCH}_2\text{C(CH}_3\text{)}_2\text{CH}_2\text{OCOC(CH}_3\text{)=CH}_2$   
 $\text{C}_8\text{F}_{17}\text{SO}_2\text{N(C}_2\text{H}_5\text{)C}_4\text{H}_8\text{OCOCH=CH}_2$   
 $(\text{C}_3\text{F}_7)_2\text{C}_6\text{H}_3\text{SO}_2\text{N(CH}_3\text{)C}_2\text{H}_4\text{OCOCH=CH}_2$   
 $\text{C}_8\text{F}_{17}\text{CF=CHCH}_2\text{N(CH}_3\text{)C}_2\text{H}_4\text{OCOCH=CH}_2$   
 as discussed in U.S. Pat. No. 5,380,644, incorporated by reference herein.

The vinyl polymers according to the present invention may be prepared by conventional solution polymerization

methods, bulk polymerization methods, emulsion polymerization methods, suspension polymerization methods, or dispersion polymerization methods. The polymerization process is initiated in general with free radical initiators. Free radicals of any sort may be used. Preferred initiators include persulfates (such as ammonium persulfate, potassium persulfate, etc., peroxides (such as hydrogen peroxide, benzoyl peroxide, cumene hydroperoxide, tertiary butyl peroxide, etc.), azo compounds (such as azobiscyanovaleric acid, azoisobutyronitrile, etc.), and redox initiators (such as hydrogen peroxide-iron (II) salt, potassium persulfate-sodium hydrogen sulfate, etc.). Common chain transfer agents or mixtures thereof known in the art, such as alkyl-mercaptans, can be used to control the polymer molecular weight.

When solution polymerization is employed, examples of suitable solvent medium include ketones such as methyl ethyl ketone, methyl butyl ketone, esters such as ethyl acetate, butyl acetate, ethers such as ethylene glycol monobutyl ether, and alcohols such as 2-propanol, and 1-butanol.

The vinyl polymers useful for the present invention include those described in U.S. Pat. Nos. 5,597,680 and 5,597,681.

In a particularly preferred embodiment, the photographic elements of this invention are photographic films, photographic papers or photographic glass plates, in which the image-forming layer is a radiation-sensitive silver halide emulsion layer. Such emulsion layers typically comprise a film-forming hydrophilic colloid. The most commonly used of these is gelatin and gelatin is a particularly preferred material for use in this invention. Useful gelatins include alkali-treated gelatin (cattle bone or hide gelatin), acid-treated gelatin (including pigskin gelatin) and gelatin derivatives such as acetylated gelatin, phthalated gelatin and the like. Other hydrophilic colloids that can be utilized alone or in combination with gelatin include dextran, gum arabic, zein, casein, pectin, collagen derivatives, collodion, agar-agar, arrowroot, albumin, and the like. Still other useful hydrophilic colloids are water-soluble polyvinyl compounds such as polyvinyl alcohol, polyacrylamide, poly(vinylpyrrolidone), and the like.

The photographic elements of the present invention can be simple black-and-white or monochrome elements comprising a support bearing a layer of light-sensitive silver halide emulsion or they can be multilayer and/or multicolor elements.

Color photographic elements of this invention typically contain dye image-forming units sensitive to each of the three primary regions of the spectrum. Each unit can be comprised of a single silver halide emulsion layer or of multiple emulsion layers sensitive to a given region of the spectrum. The layers of the element, including the layers of the image-forming units, can be arranged in various orders as is well known in the art.

A preferred photographic element according to this invention comprises a support bearing at least one blue-sensitive silver halide emulsion layer having associated therewith a yellow image dye-providing material, at least one green-sensitive silver halide emulsion layer having associated therewith a magenta image dye-providing material and at least one red-sensitive silver halide emulsion layer having associated therewith a cyan image dye-providing material.

In addition to emulsion layers, the elements of the present invention can contain auxiliary layers conventional in photographic elements, such as overcoat layers, spacer layers, filter layers, interlayers, antihalation layers, pH lowering

layers (sometimes referred to as acid layers and neutralizing layers), timing layers, opaque reflecting layers, opaque light-absorbing layers and the like. The support can be any suitable support used with photographic elements. Typical supports include polymeric films, paper (including polymer-coated paper), glass and the like. Details regarding supports and other layers of the photographic elements of this invention are contained in Research Disclosure, Item 36544, September, 1994 and Research Disclosure, Item 38957 September 1996 herein incorporated by reference.

The light-sensitive silver halide emulsions employed in the photographic elements of this invention can include coarse, regular or fine grain silver halide crystals or mixtures thereof and can be comprised of such silver halides as silver chloride, silver bromide, silver bromoiodide, silver chlorobromide, silver chloroiodide, silver chlorobromoiodide, and mixtures thereof. The emulsions can be, for example, tabular grain light-sensitive silver halide emulsions. The emulsions can be negative-working or direct positive emulsions. They can form latent images predominantly on the surface of the silver halide grains or in the interior of the silver halide grains. They can be chemically and spectrally sensitized in accordance with usual practices. The emulsions typically will be gelatin emulsions although other hydrophilic colloids can be used in accordance with usual practice. Details regarding the silver halide emulsions are contained in Research Disclosure, Item 36544, September, 1994, and the references listed therein.

The photographic silver halide emulsions utilized in this invention can contain other addenda conventional in the photographic art. Useful addenda are described, for example, in Research Disclosure, Item 36544, September, 1994. Useful addenda include spectral sensitizing dyes, desensitizers, antifoggants, masking couplers, DIR couplers, DIR compounds, antistain agents, image dye stabilizers, absorbing materials such as filter dyes and UV absorbers, light-scattering materials, coating aids, plasticizers and lubricants, and the like.

Depending upon the dye-image-providing material employed in the photographic element, it can be incorporated in the silver halide emulsion layer or in a separate layer associated with the emulsion layer. The dye-image-providing material can be any of a number known in the art, such as dye-forming couplers, bleachable dyes, dye developers and redox dye-releasers, and the particular one employed will depend on the nature of the element, and the type of image desired. Dye-image-providing materials employed with conventional color materials designed for processing with separate solutions are preferably dye-forming couplers; i.e., compounds which couple with oxidized developing agent to form a dye. Preferred couplers which form cyan dye images are phenols and naphthols. Preferred couplers which form magenta dye images are pyrazolones and pyrazolotriazoles. Preferred couplers which form yellow dye images are benzoylacetanilides and pivalylacetanilides.

A preferred photographic element according to the present invention comprises one or more silver halide light sensitive emulsion layers on one side of the support and the said backing protective layer present on the other side of the support as an outermost backing layer, or an outermost protective layer on the top of an abrasion resistance backing layer, or an outermost layer coated on the top of an antistatic layer, or an outermost layer coated on an magnetic recording layer. The backing protective layer can also comprise a lubricant.

According to a first embodiment said backside protective overcoat is applied on a support surface which is un-subbed

or subbed with an adhesion promotion layer (primer layer). The unsubbed or subbed support surface can be pre-modified with treatment such as, for example, corona discharge, plasma, solvent etching, and the like.

According to a second embodiment said backside protective overcoat is applied on a support which employs an abrasion resistant backing layer that comprises, for example, an acrylic polymer, a cellulose derivative, a polyurethane, a mixture of film-forming and non-film forming polymer particles, a sol-gel material, and the like. Such abrasion resistant layer compositions have been described in, for example, U.S. Pat. Nos. 4,582,784, 5,045,394, 5,232,824, and 5,447,832.

According to a third embodiment said backside protective overcoat is applied on a support which contains an antistatic layer that comprises, for example, a highly crosslinked vinylbenzyl quaternary ammonium polymer and a hydrophobic binder described in U.S. Pat. No. 4,070,189, a highly conductive colloidal vanadium pentoxide described in U.S. Pat. Nos. 4,203,769, and 5,006,451, a conductive fine particle of crystalline metal oxides and a film-forming binder, a conductive metal antimonate and a film-forming binder described in U.S. Pat. No. 5,368,995, and the like.

According to a fourth embodiment said backside protective overcoat is applied on a support which contains a magnetic recording layer as described in, for example, U.S. Pat. No. 4,990,276; Research Disclosure, Item 34390, November 1992; and U.S. Pat. Nos. 5,395,743, 5,397,826, 5,113,903, 5,432,050, 5,434,037, and 5,436,120.

Another preferred imaging element according to the present invention comprises one or more silver halide emulsion layers on one side of the support and on the other side of the support the backside protective overcoat of the invention. The backside protective overcoat is used as an abrasion resistant backing layer, or an antistatic layer when it is applied together with an antistatic agent, or a magnetic recording layer when it is applied together with a magnetic recording particle.

A separate lubricant layer can be applied on the top of the backside protective overcoat of the invention. Lubricants which are useful for the practice of the invention include: (1) silicone based materials disclosed, for example, in U.S. Pat. Nos. 3,489,567, 3,080,317, 3,042,522, 4,004,927, and 4,047,958, and in British Pat. Nos. 955,061 and 1,143,118; (2) higher fatty acids and derivatives, higher alcohols and derivatives, metal salts of higher fatty acids, higher fatty acid esters, higher fatty acid amides, polyhydric alcohol esters of higher fatty acids, etc disclosed in U.S. Pat. Nos. 2,454,043, 2,732,305, 2,976,148, 3,206,311, 3,933,516, 2,588,765, 3,121,060, 3,502,473, 3,042,222, and 4,427,964, in British Pat. Nos. 1,263,722, 1,198,387, 1,430,997, 1,466, 304, 1,320,757, 1,320,565, and 1,320,756, and in German Pat. Nos. 1,284,295 and 1,284,294; (3) liquid paraffin and paraffin or wax like materials such as carnauba wax, natural and synthetic waxes, petroleum waxes, mineral waxes and the like; (4) perfluoro- or fluoro- or fluorochloro-containing materials, which include poly(tetrafluoroethylene), poly(trifluorochloroethylene), poly(vinylidene fluoride), poly(trifluorochloroethylene-co-vinyl chloride), poly(meth)acrylates or poly(meth)acrylamides containing perfluoroalkyl side groups, and the like.

As the organic solvent, any of the members customarily used in coating compositions may be satisfactorily used. However, the preferred solvents for the practice of the present invention may include, for example, acetone, MEK, methanol, ethanol, butanol, dowanol PM, iso-propanol, propanol, toluene, xylene, MIBK, and their mixtures.

Among all the solvents, acetone, methanol, ethanol, iso-propanol, dowanol PM, butanol, and propanol are most preferred.

The coating composition in accordance with the invention may also contain suitable crosslinking agents which can react with carboxylic acid groups including epoxy compounds, polyfunctional aziridines, methoxyalkyl melamines, triazines, polyisocyanates, carbodiimides, and the like.

The coating composition of the invention can be applied by any of a number of well-known techniques, such as dip coating, rod coating, blade coating, air knife coating, gravure coating and reverse roll coating, extrusion coating, slide coating, curtain coating, and the like. After coating, the layer is generally dried by simple evaporation, which may be accelerated by known techniques such as convection heating. Known coating and drying methods are described in further detail in Research Disclosure No. 308119, Published Dec. 1989, pages 1007 to 1008.

The following examples are provided to illustrate the present invention in great detail, but in no way are intended to limit the scope thereof.

Vinyl polymers used in the example coatings are listed in Table 1 together with their composition (weight percent) and acid number. In Table 1, MMA is methyl methacrylate, EGD is ethylene glycol dimethacrylate, MA is methacrylic acid, AM is allyl methacrylate, EA is ethyl acrylate, and Zonyl TM is a fluoromonomer sold by DuPont de Nemours and Co.

TABLE 1

| Polymer | Composition                                                       | Acid Number |
|---------|-------------------------------------------------------------------|-------------|
| P-1     | Core/shell particle                                               | 19.5        |
|         | Core/shell: 70/30                                                 |             |
|         | Core: MMA:EGD:AM = 85:10:5<br>Shell: MMA:MA = 90:10               |             |
| P-2     | Core/Shell particle                                               | 0           |
|         | Core/shell: 50/50<br>Core: EA:BGD:AM = 94:1:5<br>Shell: MMA = 100 |             |
| P-3     | Poly(MMA-co-MA)<br>MMA:MA = 90: 10                                | 65          |
| P-4     | Poly(MMA-co-MA)<br>MMA:MA = 87.5:12.5                             | 81          |
| P-5     | Poly(MMA-co-MA)<br>MMA:MA = 85: 15                                | 98          |
| P-6     | Poly(MMA-co-MA-co-Zonyl TM)<br>MMA:MA:Zonyl TM = 60:15:25         | 98          |

P-1 and P-2 are prepared according to procedures described in U.S. Pat. No. 5,597,680. P-3 through P-6 are prepared by emulsion polymerization. Resultant polymers are isolated, washed, and dried before use.

#### EXAMPLES 1 to 16

Coating formulations in acetone/methanol solvent mixtures comprising 5 wt % total solids are applied onto cellulose acetate support which has previously been coated with a vanadium pentoxide/cellulose nitrate containing antistatic layer prepared according to Example 1B of U.S. Pat. No. 5,356,468. The coatings are dried at 100° C. for one minute to give transparent films with a dry coating weight of 1 g/m<sup>2</sup>.

It is known (described in U.S. Pat. Nos. 5,006,451 and 5,221,598) that the antistatic properties of the vanadium pentoxide layer are destroyed after photographic processing if not protected by an impermeable barrier. Thus the permeability of the example coatings can be evaluated by

measuring the antistatic properties of the elements after processing in conventional C-41 photographic processing solutions. The internal resistivity (using the salt bridge method, described in R. A. Elder, "Resistivity Measurements on Buried Conductive Layer's", EOS/ESD Symposium Proceedings, Sept. 1990, pages 251-254.) of the processed elements at 50% relative humidity is measured and compared with the internal resistivity before processing. The results are given in Table 2.

The surface haze or scum formation propensity is tested as follows: The example coatings are first processed in a C-41 processor and the dry processed strips are dipped in a C-41 stabilizer solution doctored with 500 ppm  $\text{CaCO}_3$  equivalent, prepared by adding  $\text{CaCl}_2 \cdot 2\text{H}_2\text{O}$  and  $\text{NaHCO}_3$  to the stabilizer solution. After dipping, the strips are hung to air-dry without rinsing or squeegeeing to remove excess liquid. The dried strips are evaluated under reflected and transmitted light for the presence of surface haze or scum. In Table 2, "none" refers to no scum or surface haze observed on the example coating surface, and "heavy" refers to heavy scum or surface haze observed on the example coating surface.

The scratch resistance of the example coatings is evaluated by the Taber Abrasion test in accordance with the procedure set forth in ASTM D1044. "Excellent" refers to lower amounts of transmitted haze after Taber abrasion testing while "good" refers to higher haze levels.

The examples show that the coating compositions of the invention provide highly transparent films with excellent resistance to surface haze or scum formation during photographic processing, excellent scratch resistance, and excellent protection to an underlying antistatic layer from attack by film processing solutions. Example 16 shows that a film prepared according to U.S. Pat. No. 4,735,976 provides resistance to surface haze or scum, but does not provide protection to an underlying antistatic layer.

TABLE 2

| Coatings                  | Com-<br>position            | Internal Resistivity<br>$\log \Omega/\square$ |                          |       | Scum or<br>Surface<br>Haze | Scratch<br>Resistance |
|---------------------------|-----------------------------|-----------------------------------------------|--------------------------|-------|----------------------------|-----------------------|
|                           |                             | Before<br>C-41<br>Processing                  | After C-41<br>Processing |       |                            |                       |
| Example 1<br>(Comparison) | P-1                         | 6.6                                           | 6.5                      | Heavy | Excellent                  |                       |
| Example 2<br>(Comparison) | P-2                         | 6.6                                           | 6.7                      | Heavy | Good                       |                       |
| Example 3<br>(Comparison) | P-2/P-5<br>80/20<br>(wt/wt) | 6.6                                           | >12.5                    | None  | Good                       |                       |
| Example 4<br>(Comparison) | P-2/P-4<br>70/30<br>(wt/wt) | 6.6                                           | >12.5                    | None  | Good                       |                       |
| Example 5<br>(Comparison) | P-2/P-5<br>70/30<br>(wt/wt) | 6.6                                           | >12.5                    | None  | Good                       |                       |
| Example 6<br>(Comparison) | P-1/P-6<br>98/2<br>(wt/wt)  | 6.6                                           | 6.5                      | Heavy | Excellent                  |                       |
| Example 7<br>(Comparison) | P-1/P-3<br>80/20<br>(wt/wt) | 6.6                                           | 6.6                      | Heavy | Excellent                  |                       |
| Example 8<br>(Comparison) | P-1/P-3<br>70/30<br>(wt/wt) | 6.6                                           | 6.8                      | Heavy | Excellent                  |                       |
| Example 9<br>(Invention)  | P-1/P-6<br>90/10<br>(wt/wt) | 6.6                                           | 7.3                      | None  | Excellent                  |                       |
| Example 10                | P-1/P-4                     | 6.6                                           | 6.6                      | None  | Excellent                  |                       |

TABLE 2-continued

| Coatings     | Com-<br>position            | Internal Resistivity<br>$\log \Omega/\square$ |                          |  | Scum or<br>Surface<br>Haze | Scratch<br>Resistance |
|--------------|-----------------------------|-----------------------------------------------|--------------------------|--|----------------------------|-----------------------|
|              |                             | Before<br>C-41<br>Processing                  | After C-41<br>Processing |  |                            |                       |
| (Invention)  | 80/20<br>(wt/wt)            |                                               |                          |  |                            |                       |
| Example 11   | P-1/P-4                     | 6.6                                           | 6.7                      |  | None                       | Excellent             |
| (Invention)  | 75/25                       |                                               |                          |  |                            |                       |
| Example 12   | P-1/P-4                     | 6.6                                           | 6.7                      |  | None                       | Excellent             |
| (Invention)  | 70/30<br>(wt/wt)            |                                               |                          |  |                            |                       |
| Example 13   | P-1/P-5<br>85/15<br>(wt/wt) | 6.6                                           | 6.8                      |  | None                       | Excellent             |
| (Invention)  | 80/20<br>(wt/wt)            |                                               |                          |  |                            |                       |
| Example 14   | P-1/P-5                     | 6.6                                           | 7.4                      |  | None                       | Excellent             |
| (Invention)  | 75/25                       |                                               |                          |  |                            |                       |
| Example 15   | CN/P-5<br>75/25             | 6.6                                           | 6.7                      |  | Heavy                      | Good                  |
| (Comparison) |                             |                                               |                          |  |                            |                       |
| Example 16   | CN/P-5<br>25/75             | 6.6                                           | >12.5                    |  | None                       | Good                  |
| (Comparison) |                             |                                               |                          |  |                            |                       |

25 CN is cellulose nitrate (40-60 second grade from Societe Nationale Powders and Explosives).

The invention has been described in detail with particular reference to certain preferred embodiments thereof, but it will be understood that variations and modifications can be effected within the spirit and scope of the invention.

30 What is claimed is:

1. A photographic element comprising:  
a support having a frontside and a backside;  
at least one silver halide emulsion layer superposed on the frontside of the support; and  
a protective overcoat layer superposed on the backside of the support comprising a mixture of a first vinyl polymer having an acid number of from 5 to 100 and a second vinyl polymer having an acid number of from 70 to 250 wherein the acid number of the second polymer is greater than the acid number of the first polymer wherein the first vinyl polymer further comprises fluorinated or perfluorinated vinyl monomers.
2. A photographic element comprising:  
a support having a frontside and a backside;  
at least one silver halide emulsion layer superposed on the frontside of the support; and  
a protective overcoat layer superposed on the backside of the support comprising a mixture of a first vinyl polymer having an acid number of from 5 to 100 and a second vinyl polymer having an acid number of from 70 to 250 wherein the acid number of the second polymer is greater than the acid number of the first polymer wherein the second vinyl polymer further comprises fluorinated or perfluorinated vinyl monomers.
3. The photographic element of claim 1, or 2 wherein the first vinyl polymer has an acid number of from 5 to 65.
4. The photographic element of claim 1, or 2 wherein the second vinyl polymer has an acid number of from 80 to 150.
5. The photographic element of claim 1, or 2 further comprising a weight ratio of the second vinyl polymer to the first vinyl polymer of from 5:95 to 40:60.
6. The photographic element of claim 1, or 2 wherein the second vinyl polymer has a molecular weight lower than a molecular weight of the first vinyl polymer.

**11**

7. The photographic element of claim **1**, or **2** wherein the protective overcoat layer further comprises surfactants, coating aids, matte particles, rheology modifiers, crosslinking agents, inorganic fillers, antistatic agents, pigments, magnetic particles, biocide, or lubricants.

8. The photographic element of claim **1** or **2** wherein the first and second vinyl polymers comprise a dry coverage of from 0.01 to 10 g/m<sup>2</sup>.

9. The photographic element of claim **1**, or **2** further comprising a subbing layer interposed between the support and the protective overcoat layer.

10. The photographic element of claim **1**, or **2** further comprising an abrasion resistant interposed between the support and the protective overcoat layer.

11. The photographic element of claim **1**, or **2** further comprising an antistatic layer interposed between the support and the protective overcoat layer.

5

**12**

12. The photographic element of claim **1**, or **2** further comprising a magnetic layer interposed between the support and the protective overcoat layer.

13. A photographic element comprising:  
a support having a frontside and a backside;  
at least one silver halide emulsion layer superposed on the frontside of the support; and  
a protective overcoat layer applied from an organic solvent superposed on the backside of the support comprising a mixture of a first vinyl polymer having an acid number of from 5 to 100 and a second vinyl polymer having an acid number of from 70 to 250 wherein the acid number of the second polymer is greater than the acid number of the first polymer wherein either the first or second polymer further comprises fluorinated or perfluorinated vinyl monomers.

\* \* \* \* \*